

Nov. 4, 1952

F. S. WARTMAN

**2,616,800**

## METHOD OF MAKING CUPRO-TITANIUM

Filed Nov. 22, 1949



FRANK S. WARTMAN  
INVENTOR

## INVENTOR

BY *Ray C. Hackley Jr.*  
ATTORNEY

## UNITED STATES PATENT OFFICE

2,616,800

## METHOD OF MAKING CUPRO-TITANIUM

Frank S. Wartman, Tucson, Ariz., assignor to the  
United States of America as represented by the  
Secretary of the Interior

Application November 22, 1949, Serial No. 128,897

1 Claim. (Cl. 75—164)

(Granted under the act of March 3, 1883, as  
amended April 30, 1928; 370 O. G. 757)

1

The invention described herein may be manufactured and used by or for the Government of the United States for governmental purposes without the payment to me of any royalty thereon in accordance with the provisions of the act of April 30, 1928 (Ch. 460, 45 Stat. L. 467).

This invention relates to the manufacture of metal alloys, and more particularly, to the production of alloys containing copper and titanium. Heretofore, alloys of copper and titanium have been produced by the reaction of titanic acid with a molten alloy containing copper and aluminum, for example, by the process shown in U. S. Reissue Patent No. 12,764 in the name of A. J. Rossi. Alloys of copper and titanium have great utility in the arts, not only for fabrication but also for employment as deoxidizing agents in the manufacture of copper alloys generally. Alloys of copper with titanium are also useful as master alloys for purposes of grain refinement, hardening and the like, when added to other alloys of copper. It has now been found that alloys of copper with titanium of controlled composition can be prepared by a simple and novel method susceptible of large scale operation.

Accordingly, this invention has for an object the production of alloys of copper with titanium. Another object is to prepare such alloys containing between about 22 and 27% titanium by weight which are capable of melting at a relatively low temperature. Still another object is to prepare alloys of copper with titanium by a process utilizing titanium chloride as a raw material. Further objects will be apparent or will appear as the ensuing description proceeds.

These objects are accomplished in accordance with this invention which provides a process for the production of an alloy of copper with titanium wherein an alloy of copper with magnesium is heated to fusion temperature while protecting the same from contact with the atmosphere, then titanic chloride is passed through said fused alloy in an amount sufficient to react with the magnesium metal, the reaction mass is cooled and the formed cupro-titanium is separated from the formed magnesium chloride. In one preferred embodiment the original alloy of copper with magnesium contains a sufficient quantity of magnesium such that when reacted with titanic chloride, there will result a cupro-titanium alloy containing between 22 and 27% by weight of titanium.

While it is not desired to limit the invention to any particular theory of reaction, from information presently available, it appears that the

metallic magnesium, when heated to fusion temperature in the form of an alloy with copper, reacts with titanium tetrachloride or other titanium halide, to yield a magnesium halide salt while liberating metallic titanium. Forthwith, the liberated metallic titanium alloys with the molten copper and the liberated magnesium chloride or other magnesium halide floats to the top of the fused alloy. For each percent by weight of magnesium in the original copper-magnesium alloy, there results 0.986% by weight of metallic titanium in the final copper-titanium alloy produced, provided, of course, that sufficient titanium chloride is passed into the cupro-magnesium alloy to react completely with the magnesium content thereof. Preferably, in the preparation of cupro-titanium in accordance with this invention, a slight excess of titanium tetrachloride is introduced into the molten cupro-magnesium alloy, say 1% excess, in order to insure substantially complete reaction of the magnesium content.

During the course of the reaction between the copper-magnesium alloy and the introduced titanium tetrachloride, it is necessary to protect the fused metallic mass from contact with the atmosphere or other contaminating gases. As is known, titanium rapidly reacts with such diverse gases as oxygen, nitrogen, hydrogen, carbon monoxide, carbon dioxide and the like. Accordingly, the reaction mixture is enveloped in an inert gas, by preference one of the so-called "rare" gases: argon, krypton, and preferably helium, may be employed as a protective atmosphere since none of these gases substantially react with magnesium or titanium. Similarly, the heated reaction mixture must be protected from contact with metals, otherwise the cupro-titanium and cupro-magnesium alloys will, in turn, alloy with metallic components. Since titanium tetrachloride is highly corrosive to metals generally, it is desirable that the reaction mixture and heated conduits through which titanium tetrachloride is introduced be made of graphite or other inert refractory materials.

Reference is made to the accompanying drawing wherein is shown an elevation partly in section of apparatus suitable for carrying out the production of cupro-titanium in accordance with this invention. In the drawing is shown a closed furnace 1 having a burner 2 for admission of air and fluid fuel. Near the lower portion of the furnace 1 there is shown a port 3 from which is withdrawn the produced cupro-titanium and magnesium chloride, as will be described in more

detail hereinafter. A flue 4 in the upper portion of the furnace 1 permits spent combustion gases to emerge. Axially positioned in the furnace 1 is a metallic receptacle 5 supported by a refractory column 6 resting on the bottom of the furnace 1. The receptacle 5 is provided with a graphite lining 7 which is drawn out to form a tapping spout 8 horizontally projecting therefrom at the bottom thereof. The spout 8 during heating of the charge is surrounded by a toroidal manifold 9 provided with apertures about its inner periphery for cooling the spout 8 with cold air. The manifold 9 is attached to and supported by an air pipe 10. During tapping of the charge there is utilized a launder 11 which is removable and employed only during tapping. Projecting from the receptacle 5 is a closed cylinder 12 which extends upwardly out through the top of the furnace 1 and provides a chamber for the admission of helium or other inert gas into the receptacle 5. Surrounding the cylinder 12 at the top of the furnace is a water jacket 13 provided with an inlet pipe 14 and an outlet pipe 15 for passage of water or other cooling fluid therethrough. A metal pipe 16 projects upwardly from the cylinder 12 and is positioned axially therein to provide for the admission of helium and titanium chloride into the receptacle 5. The pipe 16 terminates at the upper portion of the furnace 1 but is continued by a graphite tube 17 which extends nearly to the bottom of the receptacle 5 so as to introduce titanium tetrachloride or helium at the bottom of the receptacle 5. The pipe 16 is terminated at its upper end by a valved inlet 18 for the initial admission of helium or other insert gas into the receptacle 5 whereby air is displaced. Radially projecting from the cylinder 12 above the water jacket 13 is a valved outlet 19 for withdrawal of air and excess helium from the receptacle 5 and the cylinder 12. An additional valved inlet 20 projects from the top of the cylinder 12 for the admission of helium simultaneously with the admission of titanium tetrachloride through the pipe 16. Above the top of the cylinder 12 a valved inlet pipe 21 projects radially from the pipe 16 below the valved inlet 18 in order to introduce titanium tetrachloride into the pipe 16 through the graphite tube 17 into the receptacle 5. A flow meter 22 may be provided in the inlet pipe 21 for metering the flow of titanium tetrachloride. A tank 23 adapted to contain titanium tetrachloride is supported on weighing scales 24 and connected by means of a flexible tube 25 through the flow meter 22 to the valved inlet 21.

In operation of the above described apparatus, the furnace 1 is heated by the burner 2 while the tap hole 8 is cooled by means of air coming through the pipe 10 and being directed against the tap hole 8 by the toroidal manifold 9. For initial operation, a quantity of magnesium chloride is introduced into the receptacle 5 where it is melted and a gob thereof is solidified in the tap hole 8 by means of the air jet manifold 9. Thus, the receptacle 5 may now be charged with cupro-magnesium. The top cover 26 on the cylinder 12 is removed and granulated cupro-magnesium alloy is dropped through the cylinder 12 into the receptacle 5. Thereupon the cover 26 is replaced, the cooling jacket 13 is provided with a circulation of water or other cooling fluid and helium is passed into the valve inlet 18. At this time, the titanium tetrachloride inlet 21 is closed, as is the inlet 20, and the outlet 19 is opened. It will be seen that helium passes downwardly through the pipe 16 and the tube 17 to the bot-

tom of the receptacle 5 and the air in the receptacle 5 is displaced out of the apparatus through the outlet 19. Upon heating to a suitable temperature of say 950° C., the cupro-magnesium alloy in the receptacle 5 becomes molten. Thereupon, valved inlet 21 is opened to permit the ingress of titanium tetrachloride from the storage tank 23 through the flow meter 22 and thence downwardly through the pipe 16 to the bottom of the receptacle 5. The titanium tetrachloride forthwith reacts with the fused metal and converts the magnesium content thereof to magnesium chloride which floats above the metal as an upper layer 27. As required in order to maintain a slight pressure, additional helium is introduced through the inlet 20 concurrently with the introduction of titanium tetrachloride. The rate of introduction of titanium tetrachloride is controlled by means of the scales 24 and the flow meter 22 in order to maintain complete reaction in the receptacle 5. Generally, the receptacle 5 is heated for about an hour after the required quantity of titanium tetrachloride has been passed into the fused metal. Upon completion of the reaction, the air supply to the inlet 10 and toroidal manifold 9 is shut off and the launder 11 is inserted into the furnace so that the tap hole 8 will discharge its contents through the launder 11 into the receiver 28. As soon as the plug of magnesium chloride in the tap hole 8 melts, it, together with the product, cupro-titanium alloy, passes out through the tap hole 8 into the launder 11 and thence to the receiver 28. The operator upon observing that all of the metal and most of the magnesium chloride have been discharged, again starts the flow of cooling air through the air inlet 10 and the cycle is ready for repetition.

The following data represents a typical run in accordance with the above-described procedure:

Table

|                                                       |          |
|-------------------------------------------------------|----------|
| Pounds cupro-magnesium charged.....                   | 50       |
| Time required for bringing to temperature.....        | hours 2½ |
| Time required for addition of TiCl <sub>4</sub> ..... | do 1     |
| Pounds TiCl <sub>4</sub> added.....                   | 45       |
| Pounds cupro-titanium made.....                       | 49       |
| Analysis of alloy made:                               |          |

| Element.....           | Cu   | Ti | Fe  | Mg  | C    |
|------------------------|------|----|-----|-----|------|
| Percent by weight..... | 77.7 | 22 | 0.2 | 0.1 | 0.04 |

While the technique and apparatus described above have proved quite suitable for the intermittent operations used in developing the process, many variations come to mind which might be desirable in steady operation. Time might be saved by adding the charge of cupro-magnesium to the reaction chamber as soon as the products of the previous run had been removed and the tap hole plugged. The charge of cupro-magnesium might even be added in fluid condition by having a bath of it ready and molten in a second furnace. The tight cover and protective atmosphere of helium described might be dispensed with and a loose cover and thick fused layer of low melting chlorides used as a protective cover. For continuous operation it probably would also be advantageous to substitute an alloy resistant to oxidation at high temperatures for the mild steel used for the outer shell of the reaction chamber.

While the above description embodies the principle of the invention in its presently visualized preferred embodiment, various changes may be made as will occur to one skilled in the art with-

out departing from the spirit and scope of the invention.

What is claimed is:

A cyclic process for the production of a cupro-titanium alloy that consists in heating a vessel having a bottom tap hole, establishing a body of molten magnesium chloride therein and cooling the tap hole portion of the vessel to solidify part of the magnesium chloride therein and thus seal the tap hole; introducing a body of copper magnesium alloy into the vessel, blanketing said alloy with inert material and continuing to heat the vessel while cooling the tap hole portion thereof to establish a hot pool of fused alloy in the bottom of the vessel; passing into the fused alloy 15 a quantity of liquid titanium tetrachloride in slight stoichiometric excess with respect to the magnesium of the alloy and continuing to heat the charge until the magnesium of the alloy is converted to magnesium chloride; discontinuing 20 the cooling of the tap hole portion of the vessel to

10

5

unseal the same and drawing off through the unsealed tap hole the resulting cupro-titanium alloy and part of the supernatant magnesium chloride; re-cooling the tap hole portion of the vessel to again seal the tap hole by solidifying part of the residual supernatant magnesium chloride therein; and repeating the steps performed after the previous sealing of the tap hole.

FRANK S. WARTMAN.

#### REFERENCES CITED

The following references are of record in the file of this patent:

#### UNITED STATES PATENTS

| Number    | Name          | Date          |
|-----------|---------------|---------------|
| 1,321,684 | Turner et al. | Nov. 11, 1919 |
| 1,648,954 | Marden        | Nov. 15, 1927 |
| 2,157,979 | Cooper et al. | May 9, 1939   |
| 2,193,363 | Adamoli       | Mar. 12, 1940 |
| 2,205,854 | Kroll         | June 25, 1940 |